

1

3,148,067

PHOTOGRAPHIC SILVER HALIDE EMULSIONS  
STABILIZED WITH PYRYLUM COMPOUNDS  
George A. Reynolds, Rochester, N.Y., assignor to Eastman Kodak Company, Rochester, N.Y., a corporation of New Jersey  
No Drawing. Filed June 22, 1962, Ser. No. 204,590  
10 Claims. (Cl. 96—109)

This invention relates to photographic silver halide emulsions stabilized with certain heterocyclic compounds and to methods of preparing such emulsions.

It is well known that photographic emulsions on storage tend to lose sensitivity and to become spontaneously developable without exposure to light. There is normally a detectable amount of the silver salt reduced during development in the areas where no exposure was given; this is commonly called "fog" and sometimes called "chemical fog" where it is necessary to distinguish between it and the effects of accidental exposure to radiation; in this invention, we are not concerned with the latter.

Fog depends both on the emulsion and the conditions of development; for a given emulsion it increases with the degree of development. With constant development conditions, it tends to increase with time, temperature and relative humidity of storage conditions; it is common practice to make accelerated tests of the stability of photographic emulsions by storage at increased temperature or humidity, or both. It is, of course, desirable to have emulsions as stable as possible under the conditions of high temperature and humidity which may occur in tropical climates for example. Fog usually appears over the whole area of the sensitive coating, but when severe, it frequently is non-uniform. Fog may also be caused by exposure to chemicals, for example, hydrogen sulfide and other reactive sulfur compounds, hydrogen peroxide vapor, and strongly reducing materials. While antifoggants and stabilizers may protect, to some extent, against such effects, it is normally understood that an antifoggant protects against spontaneous growth of fog during prolonged storage or storage at high temperatures and humidities, or during development to maximum contrast and speed, or both.

It is, therefore, an object of my invention to provide a method of stabilizing photographic silver halide emulsions. A further object is to maintain the sensitivity and fog of such silver halide emulsions at, or close to, initial optimum values under keeping conditions of high temperatures and humidity. Other objects will become apparent from a consideration of the following description and examples.

According to my invention, photographic silver halide emulsions can be stabilized against the formation of spontaneous fog by incorporating in the emulsions certain pyrylium salts. Such pyrylium salts which can be usefully employed in my invention include those represented by the following general formula:

(I)



wherein R<sub>1</sub>, R<sub>2</sub> and R<sub>3</sub> each represents an aliphatic radical, such as methyl, ethyl, n-propyl, isopropyl, n-butyl, isobutyl, tertiarybutyl, n-hexyl, n-octyl, isoctyl, n-nonyl, decyl, etc. (e.g., alkyl containing from 1 to 10 carbon atoms), alkoxy, such as methoxyl, ethoxyl, propoxyl, butoxyl, pentoxyl, etc. (e.g., alkoxy containing from 1 to 5 carbon atoms), hydroxyl, etc., or an aryl radical, such as phenyl, o-, m-, and p-tolyl, o-, m-, and p-hydroxyphenyl,

2

alkoxyphenyl (e.g., p-methoxyphenyl), etc., provided at least 2 of said R radicals are alkyl, and X represents an acid anion, such as a water-solubilizing type, e.g., chloride, bromide, perchlorate, p-toluenesulfonate, methosulfate, etc.

The pyrylium compounds represented by the above general formula are quite unique in their stabilizing or antifoggant properties, since it has been found that closely related compounds do not have such useful properties. 10 For example, compounds, wherein 2 or 3 of the R radicals are aryl, are very strong desensitizers. Moreover, related compounds which contain a sulfur atom in the position occupied by the oxygen atom in the above structure do not have the useful antifoggant or stabilizing properties demonstrated by the useful pyrylium compounds of the present invention.

The compounds of Formula I above can be prepared according to a number of general methods, including the following illustrative ones:



Other anionic derivatives of these compounds can be prepared, for example, by merely treating the Grignard intermediate of Procedure B with an acid (anion of acid becomes X in formula). Procedure C can be used to prepare alkyl sulfate salts, which can be converted to less soluble forms easily. Procedure D yields  $\text{AlCl}_4^-$ ,  $\text{BF}_4^-$  and  $\text{SO}_4^{2-}$  salts. Other methods of preparing these compounds are illustrated in the copending application of J. A. Van Allan, C. C. Natale and F. J. Rauner, Serial No. 146,743, filed October 23, 1961. Typical pyrylium salts which can be used in my invention include the following: 2,6-dimethyl-4-methoxypyrylium perchlorate

65

(I)



70

## 3

2,6-dimethyl-4-ethoxypyrylium perchlorate

(2)



2,6-dimethyl-4-hydroxypyrylium perchlorate

(3)



2,4,6-trimethylpyrylium perchlorate

(4)



2,6-dimethyl-4-phenylpyrylium perchlorate

(5)



2,6-diisopropyl-4-methylpyrylium perchlorate

(6)



2,6-dimethyl-4-amylpyrylium perchlorate

(7)



4-acetoxy-2,6-dimethylpyrylium fluoroborate

(8)



4-butoxy-2,6-dimethylpyrylium perchlorate

(9)



Several of the above specific pyrylium salts have been described in the literature. Literature references for a number of these and preparative data for several others are listed below.

2,6-dimethyl-4-methoxypyrylium perchlorate: J. Chem. Soc. (1946), 117.

2,6-dimethyl-4-ethoxypyrylium perchlorate: A mixture of 12 g. of 2,6-dimethyl-4-pyrone, 20 g. of diethyl sulfate, and 1.5 ml. of ethanol was warmed at 50° C. until complete solution resulted. The solution was cooled to

## 4

room temperature, 50 g. of 20 percent aqueous perchloric acid added, and after chilling, the long white needles were collected, M.P. 215-6° C. (yield=6 g.). The reported melting point is 126-7° C.; J. Chem. Soc. (1946), 117.

5 2,6-dimethyl-4-hydroxypyrylium perchlorate: A solution of 2 g. 2,6-dimethyl-4-pyrone in 100 ml. of ether was saturated with hydrogen chloride. The 2,6-dimethyl-4-hydroxypyrylium chloride that separated was collected on a Büchner funnel and washed with ether. To a concentrated solution of the pyrylium chloride in alcohol was added 2 ml. of 70 percent perchloric acid and the mixture chilled. The product was collected and washed with ether (yield=2.2 g.).

10 2,4,6-trimethylpyrylium perchlorate: Ber., 60, 722 (1927).

15 2,6-dimethyl-4-phenylpyrylium perchlorate: Ann., 432, 297 (1923).

2,6-diisopropyl-4-methylpyrylium perchlorate: Ann., 625, 74 (1959).

20 2,6-dimethyl-4-amylpyrylium perchlorate: A solution of amylmagnesium bromide (prepared from 15 g. of 1-bromopentane, 2.4 g. of magnesium and 100 ml. of ether) was added slowly with cooling and stirring to 14 g. of 2,6-dimethyl-4-pyrone in 250 ml. of dry tetrahydrofuran. The mixture was stirred for one hour and then acidified with aqueous perchloric acid. The reaction mixture was concentrated at room temperature to half volume and then chilled to yield 4 g. of product as long white needles, M.P. 180° C.

25 30 The stabilizing compounds of my invention are particularly useful in photographic developing-out emulsions, including many of the conventionally employed silver halide emulsions, such as silver chloride, silver bromide, silver bromide, silver chlorobromide, silver chloro-bromide, etc.

The emulsions can be chemically sensitized by any of the accepted procedures. The emulsions can be digested with naturally active gelatin, or sulfur compounds can be added such as those described in Sheppard U.S. Patent

40 1,574,944, issued March 2, 1926, Sheppard et al. U.S. Patent 1,623,499, issued April 5, 1927, and Sheppard et al. U.S. Patent 2,410,689, issued November 5, 1946.

The emulsions can also be treated with salts of the noble metals such as ruthenium, rhodium, palladium, iridium, and platinum. Representative compounds are ammonium chloropalladate, potassium chloroplatinate, and sodium chloropalladite, which are used for sensitizing in amounts below that which produces any substantial fog inhibition, as described in Smith and Trivelli U.S. Patent 2,448,060, issued August 31, 1948, and an antifoggants in higher amounts, as described, in Trivelli and Smith U.S. Patents 2,566,245, issued August 28, 1951, and 2,566,263, issued August 28, 1951.

45 50 The emulsions can also be chemically sensitized with gold salts as described in Waller et al. U.S. Patent 2,399,083, issued April 23, 1946, and Damschroder et al. U.S. Patent 2,642,361, issued June 16, 1953. Suitable compounds are potassium chloroaurite, potassium aurithiocyanate, potassium chloroaurate, auric trichloride and 2-aurosulfobenzothiazole methochloride.

60 65 The emulsions can also be chemically sensitized with reducing agents such as stannous salts (Carroll U.S. Patent 2,487,850, issued November 15, 1949), polyamines, such as diethylene triamine (Lowe and Jones U.S. Patent 2,518,698, issued August 15, 1950), polyamines, such as spermine (Lowe and Allen U.S. Patent 2,521,925, issued September 12, 1950), or bis(β-aminoethyl) sulfide and its water-soluble salts (Lowe and Jones U.S. Patent 2,521,926, issued September 12, 1950).

70 75 The emulsions can also be optically sensitized with cyanine and merocyanine dyes, such as those described in Brooker U.S. Patents 1,846,301, issued February 23, 1932; 1,846,302, issued February 23, 1932; and 1,942,854, issued January 9, 1934; White U.S. Patent 1,990,507, issued February 12, 1935; Brooker and White U.S. Patents 2,112,-

140, issued March 22, 1938; 2,165,338, issued July 11, 1939; 2,493,747, issued January 10, 1950, and 2,739,964, issued March 27, 1956; Brooker and Keyes U.S. Patent 2,493,748, issued January 10, 1950; Sprague U.S. Patents 2,503,776, issued April 11, 1950, and 2,519,001, issued August 15, 1950; Heseltine and Brooker U.S. Patent 2,666,761, issued January 19, 1954; Heseltine U.S. Patent 2,734,900, issued February 14, 1956; Van Lare U.S. Patent 2,739,149, issued March 20, 1956; and Kodak Limited British Patent 450,958, accepted July 15, 1936.

The emulsions may also contain speed increasing compounds of the quaternary ammonium type of Carroll U.S. Patent 2,271,623, issued February 3, 1942; Carroll and Allen U.S. Patent 2,288,226, issued June 30, 1942; and Carroll and Spence U.S. Patent 2,334,864, issued November 23, 1943; or the polyethylene glycol type of Carroll and Beach U.S. Patent 2,708,162, issued May 10, 1955; or the quaternary ammonium salts and polyethylene glycols of Piper U.S. Patent 2,886,437, issued May 12, 1959; as well as the thiopolymers of Graham and Sagal U.S. application Serial No. 779,839, filed December 12, 1958, and the Dann and Chechak U.S. application Serial No. 779,874, filed December 12, 1958.

In the preparation of the silver halide dispersions employed for preparing silver halide emulsions, there may be employed as the dispersing agent for the silver halide in its preparation, gelatin or some other colloidal material such as colloidal albumin, a cellulose derivative or a synthetic resin, for instance, a polyvinyl compound. Some colloids which may be used are polyvinyl alcohol or a hydrolyzed polyvinyl acetate as described in Lowe U.S. Patent 2,286,215, issued June 16, 1942; a far hydrolyzed cellulose ester such as cellulose acetate hydrolyzed to an acetyl content of 19-26% as described in U.S. Patent 2,327,808 of Lowe and Clark, issued August 24, 1943; a water-soluble ethanolamine cellulose acetate as described in Yutzy U.S. Patent 2,322,085, issued June 15, 1943; a polyacrylamide or an imidized polyacrylamide as described in Lowe, Minsk and Kenyon U.S. Patent 2,541,474, issued February 13, 1951; zein as described in Lowe U.S. Patent 2,563,791, issued August 7, 1951; a vinyl alcohol polymer

the silver halide emulsion in order to obtain optimum results. The quantity of stabilizing compound can be varied, depending somewhat upon the chemical activity of the stabilizer, the concentration of silver halide in the emulsion, coating thickness of the emulsion, and the like. In general, I have found that optimum results can be obtained at concentrations of from about 0.25 to about 6.0 grams per mole of silver halide in the emulsion.

The following examples will serve to illustrate the useful effects of the pyrylium compounds of my invention in ordinary photographic silver halide emulsions.

A high-speed gelatino-bromiodide emulsion was divided into several batches and a portion of each batch removed for purposes of serving as a control. To each of the remaining portions was added a small amount of antifogant and the batches, together with the control emulsions, coated on a conventional photographic support, such as cellulose acetate film. The coatings were then dried and exposed for  $\frac{1}{25}$  sec. in an Eastman Type Ib Sensitometer. The film samples were then developed in a conventional black-and-white developer, such as one having the following composition:

|    |                                | Grams |
|----|--------------------------------|-------|
| 25 | N-methyl-p-aminophenol sulfate | 5.0   |
|    | Sodium sulfite (desiccated)    | 100   |
|    | Sodium metaborate              | 2.0   |
|    | Sodium thiocyanate             | 1.0   |
|    | Potassium bromide              | 0.5   |
|    | Water to make 1 liter.         |       |

30 The developed emulsions were then fixed, washed and dried. The relative speed, gamma and fog for each of the coatings were then measured. A second set of coatings was prepared in exactly the same manner and these coatings were held for one week at 120° F. and 50 percent relative humidity before use. These coatings were likewise exposed, fixed, washed and dried as described above. The relative speed, gamma and fog for the incubated coatings were then measured, and the data obtained, together with the fresh tests, are given in the following table. In the table, the compound numbers correspond to those formulated above.

Table A

| Coating number | Compound No. | Cone. in grams/Ag mole | Fresh tests |       |      | 1-week incubation at 120° F. and 50% RH |       |      |
|----------------|--------------|------------------------|-------------|-------|------|-----------------------------------------|-------|------|
|                |              |                        | Rel. speed  | Gamma | Fog  | Rel. speed                              | Gamma | Fog  |
| (a)            | Control      |                        | 100         | 0.90  | 0.10 | 65                                      | 0.73  | 0.28 |
| (b)            | 1            | 3.0                    | 110         | 1.08  | 0.08 | 91                                      | 0.88  | 0.14 |
| (c)            | Control      |                        | 100         | 1.10  | 0.11 | 83                                      | 0.92  | 0.23 |
| (d)            | 5            | 0.75                   | 87          | 1.17  | 0.11 | 80                                      | 0.93  | 0.18 |
| (e)            | 5            | 3.0                    | 68          | 1.12  | 0.08 | 73                                      | 1.00  | 0.11 |
| (f)            | Control      |                        | 100         | 1.13  | 0.10 | 74                                      | 0.95  | 0.24 |
| (g)            | 4            | 1.5                    | 94          | 1.15  | 0.11 | 85                                      | 1.15  | 0.18 |
| (h)            | 4            | 3.0                    | 74          | 1.12  | 0.12 | 83                                      | 0.97  | 0.14 |
| (i)            | 7            | 3.0                    | 100         | 1.15  | 0.11 | 85                                      | 0.97  | 0.20 |
| (j)            | Control      |                        | 100         | 1.22  | 0.12 | 62                                      | 0.83  | 0.24 |
| (k)            | 3            | 0.75                   | 95          | 1.18  | 0.12 | 62                                      | 0.88  | 0.20 |
| (l)            | Control      |                        | 100         | 1.18  | 0.12 | 91                                      | 0.92  | 0.33 |
| (m)            | 2            | 3.0                    | 105         | 1.18  | 0.11 | 87                                      | 1.02  | 0.29 |

containing urethane carboxylic acid groups of the type described in Unruh and Smith U.S. Patent 2,768,154, issued October 23, 1956; or containing cyano-acetyl groups such as the vinyl alcohol-vinyl cyanoacetate copolymer as described in Unruh, Smith and Priest U.S. Patent 2,808,331, issued October 1, 1957; or a polymeric material which results from polymerizing a protein or a saturated acylated protein with a monomer having a vinyl group as described in U.S. Patent 2,852,382, of Illingsworth, Dann and Gates, issued September 16, 1958.

The pyrylium salts of my invention can be added to the emulsions during the preparation thereof, or during the final digestion or immediately prior to coating. It is essential that the stabilizing agent be thoroughly mixed with

it will be understood that variations and modifications can be effected within the spirit and scope of the invention as described hereinabove and as defined in the appended claims.

The invention has been described in detail with particular reference to preferred embodiments thereof, but it will be understood that variations and modifications can be effected within the spirit and scope of the invention as described hereinabove and as defined in the appended claims.

What I claim as my invention and desire secured by Letters Patent of the United States is:

1. A photographic silver halide emulsion containing as an antifoggant a stabilizing amount of the compound selected from those represented by the following general formula: 5



wherein R<sub>1</sub>, R<sub>2</sub> and R<sub>3</sub> each represents a radical selected 15 from the class consisting of alkyl containing from 1 to 10 carbon atoms, alkoxy containing from 1 to 5 carbon atoms, hydroxyl and aryl, provided at least 2 of said radicals represent alkyl containing from 1 to 10 carbon atoms, and X represents an anion.

2. A photographic silver halide emulsion containing a stabilizing amount of pyrylium salt selected from those represented by the following general formula: 20



wherein R<sub>1</sub>, R<sub>2</sub> and R<sub>3</sub> each represents alkyl containing 30 from 1 to 10 carbon atoms and X represents an anion.

3. A photographic silver halide emulsion containing a stabilizing amount of a pyrylium salt selected from those represented by the following general formula: 35



wherein R<sub>1</sub> and R<sub>3</sub> each represents alkyl containing from 1 to 10 carbon atoms, R<sub>2</sub> represents alkoxy containing from 1 to 5 carbon atoms and X represents an anion.

4. A photographic silver halide emulsion containing as an antifoggant a stabilizing amount of a compound selected from those represented by the following general formula: 40



wherein R<sub>1</sub> and R<sub>3</sub> each represents alkyl containing from 1 to 10 carbon atoms, R<sub>2</sub> represents aryl and X represents an anion.

5. A photographic silver halide emulsion containing a 45

stabilizing amount of a pyrylium salt selected from those represented by the following general formula:



10 wherein R<sub>1</sub> and R<sub>3</sub> each represents alkyl containing from 1 to 10 carbon atoms, R<sub>2</sub> represents hydroxyl and X represents an anion.

6. A photographic silver halide emulsion containing a stabilizing amount of the compound represented by the following formula: 5



7. A photographic silver halide emulsion containing as an antifoggant a stabilizing amount of the compound represented by the following formula: 20



8. A photographic silver halide emulsion containing a stabilizing amount of the compound represented by the following formula: 25



9. A photographic silver halide emulsion containing a stabilizing amount of the compound represented by the following formula: 30



10. A photographic silver halide emulsion containing a stabilizing amount of the compound represented by the following formula: 35



References Cited in the file of this patent

UNITED STATES PATENTS

2,461,484 Thompson Feb. 8, 1949